

# United States Patent Office

3,081,219

Patented Mar. 12, 1963

1

3,081,219  
**PREVENTION OF DEPOSITION OF PITCH  
IN PAPERMAKING**

IN PAPERMAKING  
Thomas J. Drennen, Lafayette Hill, and Louis E. Kelley,  
Wyncote, Pa., assignors to Rohm & Haas Company,  
Philadelphia, Pa., a corporation of Delaware  
No Drawing. Filed Feb. 10, 1960, Ser. No. 7,743  
7 Claims. (Cl. 162—72)

The present invention relates to the control of pitch 10 in the making of paper from sulfite pulps. This application is a continuation-in-part of our copending application Serial No. 788,523, filed January 23, 1959, now abandoned.

abandoned. The pitch in the fibers of wood pulps is associated with naturally occurring lignin dispersing agents. However, cooking and mechanical agitation which occur during the pulping by the sulfite process liberates the pitch but the natural dispersing agents liberated with the pitch are inadequate to keep the pitch from depositing, as a result of the mechanical work on the fibers, on the equipment employed in beating, hydrating, refining, bleaching, and even on the wire used for forming the sheet. Because of the tendency of the pitch to agglomerate within the pulp suspension or deposit on the surfaces of the wire or other equipment and then to break free in the form of particles of considerable size, the pitch frequently causes the formation of spots or holes in the sheet formed or may adhere to the wire or press rolls or drier rolls and cause tearing of the sheet. This results in occasional tearing of the sheet during formation or in the production of sheets with numerous imperfections. Among other consequences involved are the expense of cleaning the machinery frequently either with solvents or steam, and the loss of production during cleaning and during re-lacing operations caused by breakdown of the sheet.

Various systems have been employed heretofore for controlling the pitch in the making of paper from sulfite pulps whether bleached or unbleached or from ground-wood pulps. One way of controlling pitch heretofore employed is the introduction of diatomaceous earth, bentonite, or the like for the purpose of introducing finely-divided particles which adhere to the pitch and reduce the tackiness of its surface. Other expedients involve the addition of dispersing agents or sequestering agents. Polyphosphates such as sodium hexa-meta-phosphate have been employed. They have appreciable value when the pulp treated has a pH of about 3.5 to 4.5; but when the pulp is nearer the neutral state such as at a pH from 5.5 to 7, the beneficial effect is slight. Various dispersing agents have been employed such as the sodium salt of sulfonated formaldehyde/naphthalene condensates, but these agents have decreased effects at neutral pH values. They also are precipitated by cationic materials, such as alum and cationic urea-formaldehyde-polyamine wet-strength resins, so that pitch control suffers and the wet-strength efficiency of such resins is reduced when the latter materials are added to the pulp, as in the beating stage. There have also been suggestions to employ a mixture of an organic solvent for the pitch in conjunction with a dispersing agent, but these procedures involve the additional expenses of the organic solvent and of compounding the emulsifier therewith.

In accordance with the present invention, it has been discovered that highly effective pitch control of sulfite pulps over a wide range of pH from both neutral to acid conditions can be obtained by the introduction of relatively small amounts of a polymeric N-vinyl lactam. The polymers contain from 80 to 100% of the N-vinyl lactam and up to 20% by weight of a neutral comonomer such as a  $C_{1-18}$  ester of acrylic acid or methacrylic acid.

The polymers with which the present invention is concerned contain N-vinyl lactam units of the general formula



wherein R represents an alkylene bridge group necessary to complete a 5, 6, and 7-membered heterocyclic ring system, and R<sub>1</sub> represents either hydrogen or a methyl group. The materials characterized by

All of the specific polymeric materials characterized by the foregoing general formula are commercially available and called polymeric N-vinyl lactams. They are obtained by polymerizing organic 5, 6, and 7-membered ring compounds containing in their rings the



group, such as, for example, 1-vinyl-2-pyrrolidone, which in more recent terminology is called 1-vinyl-2-pyrrolidone, 1-vinyl-5-methyl-2-pyrrolidinone, 1-vinyl-2-piperidone, N-vinyl- $\epsilon$ -caprolactam, and the like. Depending upon the extent of polymerization, they have molecular weights ranging from 500 to 200,000. Viscosity measurements are used as an indication of the average molecular weight of the polymers which are characterized by a chain of carbon atoms to which the lactam rings are attached through their nitrogen atoms:



35 The viscosity coefficient  $K$ , which is fully described in Modern Plastics, 23, No. 3, 157-61, 212, 214, 216, 218 (1945), is calculated as follows:

$$\frac{\log_{10} \eta_{\text{rel}}}{C} = \frac{75K^2}{1 + 1.5KC} + K$$

where C is the concentration in gram per 100 cc. of polymer solution and  $\eta_{rel}$  is the ratio of the viscosity of the solution to that of pure solvent. The K values are reported as 1000 times the calculated viscosity coefficient in order to avoid the use of decimals. For the purpose of the present invention, there may be used those polymers having a K value of 10 to 100, preferably of 30 to 100 because of their viscosity at lower concentrations.

50 The preferred lactams are the N-vinyl-2-pyrrolidinones having the general formula



60 wherein R represents hydrogen or methyl group and  $R_1$  represents either hydrogen, methyl, or ethyl.

As illustrative examples of such N-vinylpyrrolidonates the following may be mentioned:

65 5-methyl-N-vinyl-2-pyrrolidinone  
 5-ethyl-N-vinyl-2-pyrrolidinone  
 3,3-dimethyl-N-vinyl-2-pyrrolidinone  
 3-methyl-N-vinyl-2-pyrrolidinone  
 70 3-ethyl-N-vinyl-2-pyrrolidinone  
 4-methyl-N-vinyl-2-pyrrolidinone  
 4-ethyl-N-vinyl-2-pyrrolidinone

Examples of the esters of acrylic acid or methacrylic acid, which acids have the generic formula



in which  $n$  is an integer having a value of 1 to 2, are those of the alkanols having from 1 to 18 carbon atoms including methanol, ethanol, n-propanol, isopropanol, n-butanol, hexanol, 2-ethylhexanol, n-octanol, lauryl alcohol, and stearyl alcohol. The cyclohexanol, benzyl alcohol, bornyl alcohol, and isobornyl alcohol esters may also be employed.

The proportion of N-vinyl lactam polymer that is required is in the range from about 0.005 to 0.2% by weight, based on the weight of fiber in the pulp. A larger amount of the polymer may be used, such as up to 0.5% by weight or more, based on the weight of fiber. However, polymers of the present invention are so efficient in their pitch-controlling action that less than 0.2% of the polymer on fiber is generally entirely adequate and the preferred range is from about 0.02 to 0.1% polymer on fiber. The present invention is applicable to any sulfite pulp whether bleached or unbleached as well as to groundwood pulps or mixtures thereof. It is applicable to such pulps whether in a neutral condition or near neutral condition in a range of pH from about 5 to 7 or in an acid condition wherein the range of pH may be from 5 down to 3.5 whether the acid condition is obtained by the introduction of a strong mineral acid such as sulfuric acid or an acidic salt such as any of the various alums including the common papermakers' alum. One of the advantages of the polymeric N-vinyl lactams of the present invention is the fact that they are unaffected by either anions or cations so that loss of pitch control is not caused by the use of alum in rosin sizing or of cationic wet-strength resins.

The polymeric N-vinyl lactam may be introduced into the pulp at any stage during the pulping operation including introduction prior to and immediately after digestion. The polymeric N-vinyl lactam may be introduced into the pulp at any stage of the papermaking process, such as during beating, in the stock-chest, or even in the headbox of the papermaking machine. It is preferred to add the polymeric N-vinyl lactam early in the pulping or papermaking stage before the pitch initially dispersed by the lignin agents liberated from the pulp during digestion is coagulated by the mechanical work performed on the pulp during the papermaking operations. The best results are thereby obtained since the N-vinyl lactam polymer is not required to redisperse 40 coagulated pitch but only to stabilize the pitch in its initially dispersed state. However, addition in the later stages is effective in controlling the pitch but a larger amount of the polymer may be required to obtain a given effect. When the addition of the polymer is made after digestion, such as from the beater up to the stockchest or headbox, the consistency of the pulp to which it is added may be from 0.01% to 6% fiber weight.

Generally pitch deposition is not a problem in a kraft pulp, but the polymers of the present invention can be applied to kraft pulps in those rare instances where pitch control is desirable.

In the following examples which are illustrative of the invention, the parts and percentages are by weight unless otherwise specifically indicated. The test method used to determine the amount of pitch deposited in the pulps of various of the following examples involves placing in a suitable vessel of 14-cm. diameter (e.g., a 3-liter glass beaker) a pulp containing a given weight of fiber in one liter of water and vibrating at a given high frequency, a smooth, 20-gage, stainless steel plate having dimensions of 7½ cm. by 9 cm. and positioned horizontally 2.5 cm. under the surface of the pulp. This plate as used herein may be attached to conventional vibrating equipment such as that known as the Boerner Oscillating Platform No.

8927, made by the A. H. Thomas Company. The apparatus used in the test also includes a collar (of 1 cm. outside diameter and 10 cm. length) on a rotating agitator shaft disposed so that the collar is at the surface of the pulp. The total weight of pitch collected on the vibrating plate and the collar is weighed to indicate the extent of deposition or control thereof. The time of agitation and vibration for the test is thirty minutes, and the temperature of the pulp during such agitation and vibration is 25° C. In all examples, the percentage of the N-vinyl lactam polymer is based on the weight of fiber (dry) in the pulp to which the polymer is added.

#### Example 1

15 0.35% by weight of a copolymer of 95% of N-vinyl-2-pyrrolidinone with 5% of ethyl acrylate is introduced into an unbleached sulfite pulp having a pH of 6.5% and a 3.5% pulp consistency. On testing with the vibrating plate, only 0.5 part of pitch is deposited per 1,000 parts of pulp (3.5% consistency), whereas several batches 20 of the untreated pulp under similar conditions deposited from 18 to 25 parts per 1,000 parts of pulp (3.5% consistency). The employment of 0.35% of the sodium salt of a sulfonated formaldehyde/naphthalene condensate 25 results in a deposit under similar conditions of 16.0 parts per 1,000 parts of pulp (3.5% consistency).

#### Example 2

30 A deposit of 0.9 part of pitch per 1,000 parts of pulp (3.5% consistency) occurs when 0.7% (on the weight of pulp) of a copolymer of 95% of N-vinyl-2-pyrrolidinone with 5% of lauryl methacrylate is employed for pitch control and tested as in Example 1. The employment of 0.7% by weight on the pulp of the sodium salt of a sulfonated formaldehyde/naphthalene condensate results in a deposit of 7 parts of pitch per 1,000 parts of pulp (3.5% consistency) at a pH of 6.5.

#### Example 3

When the test of Example 1 is repeated but substituting 0.7% of a copolymer of 95% of N-vinyl-2-pyrrolidinone and 5% of isobornyl methacrylate, only 0.7 part of pitch per 1,000 parts of pulp (3.5% consistency) is deposited.

#### Example 4

0.15% by weight, based on the weight of fiber, of a homopolymer of N-vinyl-2-pyrrolidinone having a K value of 30 is incorporated into a 3.5% consistency unbleached sulfite pulp adjusted to a pH of 4.0 by addition of sulfuric acid. When tested with the vibrating plate and agitator, no pitch deposits whereas under similar test conditions the incorporation of 0.15%, on fiber, of the sodium salt of sulfonated formaldehyde/naphthalene condensate results in the deposit of 5.3 parts of pitch per 1,000 parts of pulp and 8.0 parts of pitch is deposited per 1,000 parts of pulp under similar test conditions when no addition of a pitch control agent is made.

Reduction of pitch deposition in a paper mill operation was found practically effective even when the amount of the polymer was reduced to about 0.01 to 0.04% on the fiber weight.

#### Example 5

65 0.2% by weight of a homopolymer of N-vinyl-pyrrolidinone is introduced into an unbleached sulfite pulp having a pH of 7.0. The percentage of polymer is based on the weight of fiber solids and the consistency of the pulp is 3.5% by weight of fiber. The polymer has a K value of 30 and the 5% solution in water at 25° C. shows a viscosity of 4 cps. determined in a Brookfield viscometer at 60 r.p.m. The equipment employed in producing paper from this composition shows greatly reduced deposition of pitch as compared with the equipment when 70 paper is produced without the incorporation of the poly-

mer in the pulp. Similarly, the paper sheets show very few pitch spots of minute size when obtained with the pulp containing the polymer, whereas paper sheets obtained from the pulp without the addition of polymer have relatively numerous pitch spots ranging in size from one-fourth of a millimeter to as large as one millimeter in average diameter. Comparative testing of the pulp with and without the 0.2% of polymer on fiber shows a pitch deposit of 0.6 part of pitch per 1,000 parts of pulp in the case of the treated pulp and 5.9 parts of pitch per 1,000 parts of pulp in the case of the untreated pulp.

*Example 6*

An unbleached sulfite pulp of 3.2% consistency and having a pH of 6.7 to 8 is used for producing paper sheets. A portion of this pulp is modified by introducing into the beater 0.1% by weight, on the weight of pulp solids, of poly(N-vinyl-2-pyrrolidinone) having a K value of 60. Another portion of the pulp is used for making paper sheets without the addition of the polymer. The pitch deposition is observed at various stages during the beating with the following results. After 10 minutes of defibering (without lowering the beater roll), 0.2 part of pitch per 1,000 parts of pulp is deposited from the pulp containing the polymer, whereas 8.2 parts of pitch per 1,000 parts of pulp is deposited from the pulp which does not contain the polymer. After 30 minutes of beating, 0.7 part of pitch per 1,000 parts of pulp is deposited from the polymer-containing pulp, whereas 8.9 parts of pitch per 1,000 parts of pulp are deposited in the case of the pulp which contains no added polymer.

The paper sheets obtained from the polymer-containing pulp show fewer pitch spots which have much smaller average diameters than the sheets obtained with the untreated pulp.

We claim:

1. A paper-making composition comprising fibers from a sulfite wood pulp having a content of pitch such as to give rise normally to a pitch problem by virtue of the tendency of the pitch to agglomerate and deposit in the form of particles of considerable size when unmodified by a pitch-controlling agent, the fibers in the composition consisting exclusively of cellulose fibers, the composition having a consistency from 0.01 to 6% and containing, as a pitch-controlling material, 0.005 to 0.2% by weight, based on fiber weight, of a polymer of 80 to 100% by weight of N-vinyl-2-pyrrolidinone.

2. A composition as defined in claim 1 in which the

polymer is a copolymer containing up to 20% by weight of an ester of an acid of the formula



5 in which  $n$  is an integer having a value of 1 to 2.

3. A composition as defined in claim 1 in which the polymer is a copolymer containing up to 20% by weight of ethyl acrylate.

10 4. A composition as defined in claim 1 in which the polymer is a copolymer containing up to 20% by weight of lauryl methacrylate.

5. A composition as defined in claim 1 in which the polymer is a copolymer containing up to 20% by weight of isobornyl methacrylate.

15 6. The method of controlling pitch in making paper from fibers consisting exclusively of the cellulose fibers of a sulfite pulp having a pitch problem which comprises incorporating into the sulfite pulp from 0.005% to 0.2% by weight, based on the weight of the pulp solids, of a polymer of 80 to 100% by weight of N-vinyl-2-pyrrolidinone and up to 20% by weight of an ester of an acid of the formula



20 25 in which  $n$  is an integer having a value of 1 to 2, at a stage between the time immediately before digestion and immediately before the time of deposition of the pulp as a paper sheet, and forming a paper sheet from the pulp containing the polymer.

30 35 7. The method of controlling pitch in making paper from fibers consisting exclusively of the cellulose fibers of a sulfite pulp having a pitch problem which comprises incorporating into the sulfite pulp from 0.005% to 0.2% by weight, based on the weight of the pulp solids, of a homopolymer of N-vinyl-2-pyrrolidinone, at a stage between the time immediately before digestion and immediately before the time of deposition of the pulp as a paper sheet, and forming a paper sheet from the pulp containing the polymer.

References Cited in the file of this patent

UNITED STATES PATENTS

|    |           |          |       |               |
|----|-----------|----------|-------|---------------|
| 45 | 2,335,454 | Schuster | ----- | Nov. 30, 1943 |
|    | 2,667,473 | Morner   | ----- | Jan. 26, 1954 |
|    | 2,771,362 | Moser    | ----- | Nov. 20, 1956 |
|    | 2,901,390 | Conklin  | ----- | Aug. 25, 1959 |
|    | 2,945,863 | Buc      | ----- | July 19, 1960 |